

No. 714,861.

Patented Dec. 2, 1902.

D. H. BROWNE.

PROCESS OF ELECTROLYTIC SEPARATION OF COPPER AND NICKEL.

(Application filed Jan. 27, 1899. Renewed Sept. 18, 1902.)

(No Model.)



Witnesses,  
J. C. Turner  
D. Davies.

Inventor,  
David H. Browne

By  
Thos. Hall  
Attest.

# UNITED STATES PATENT OFFICE.

DAVID H. BROWNE, OF CLEVELAND, OHIO, ASSIGNOR TO THE CANADIAN COPPER COMPANY, OF CLEVELAND, OHIO, A CORPORATION OF OHIO.

## PROCESS OF ELECTROLYTIC SEPARATION OF COPPER AND NICKEL.

SPECIFICATION forming part of Letters Patent No. 714,861, dated December 2, 1902.

Application filed January 27, 1899. Renewed September 19, 1902. Serial No. 124,080. (No specimens.)

To all whom it may concern:

Be it known that I, DAVID H. BROWNE, a citizen on the United States, and a resident of Cleveland, county of Cuyahoga, and State of Ohio, have invented a new and useful Improvement in Processes for the Electrolytic Separation of Copper and Nickel, of which the following is a specification, the principle of the invention being herein explained and the best mode in which I have contemplated applying that principle, so as to distinguish it from other inventions.

My invention has for its object the improved separation of copper and nickel by electrolysis on a commercial scale; and it consists of a process hereinafter fully described.

In the annexed drawing is represented diagrammatically one form of apparatus adapted to be used in my process.

20 Copper-nickel matte is treated by any suitable process to form copper-nickel alloy substantially free from sulfur. From the copper-nickel alloy so procured are made in proportions dependent upon the relative amount of 25 copper and nickel therein contained copper-nickel anodes and copper-nickel fragments or powder.

The copper-nickel fragments or powder are placed in a receptacle A, which I shall designate the "shot-tower" and which is provided 30 with apertures  $a a' a''$ . Such subject-matter is there subjected simultaneously to the action of a stream of a solvent for cuprous chlorid, such as salt water, introduced into the 35 top of the tower at  $a$  and a stream of free chlorin introduced at the side of the tower through the aperture  $a'$ . The combined actions of the salt water and of the heat produced by the combination of the chlorin with 40 the copper-nickel alloy form a solution of cuprous and nickel chlorids, the reaction being



Such solution is permitted to run out through 45 the aperture  $a''$  and thence into an electrolytic cell B, containing an anode  $b$  of the copper-nickel metal and a cathode  $b'$ . The electric current being passed through the solution of cuprous and nickel chlorids, the cuprous chlorid is decomposed, the copper plating out upon the cathode, and the chlorin com-

bining with the copper and the nickel of the anode, forming cuprous chlorid and additional nickel chlorid, the reaction being



The cuprous chlorid so formed is also decomposed in the same manner as was that of the original solution, cuprous and nickel chlorids being formed from the anode as before and 60 copper plating out. In this manner all the copper is plated out and only nickel chlorid remains, which nickel chlorid is permitted to emerge from the cell, as at  $b'$ . The nickel chlorid is now freed from any impurities, 65 such as iron or traces of copper, the iron being precipitated by any alkali, which neutralizes the liquor, the reaction being



Said liquor is then heated to a temperature of between 30° and 60° centigrade and is also increased in strength, preferably to a density of from 30° to 50° Baumé. It is thereupon 75 introduced into a nickel-plating apparatus, which may consist of a series of cells, such as C, each of which may have a porous diaphragm c, an anode-cap c', a carbon anode c<sup>2</sup>, a nickel cathode c<sup>3</sup>, a chlorin-escape c<sup>4</sup> connecting with aperture  $a'$  of the shot-tower A. On the passage of an electric current through 80 this latter solution nickel is plated upon the cathode and chlorin gas is liberated at the anode, the reaction being



Said chlorin gas is thence conducted to the shot-tower A and is utilized, as previously described, to form the solution of copper and 90 nickel chlorids, the reaction being



Other modes of applying the principle of my invention may be employed instead of the 95 one explained, change being made as regards the steps herein disclosed, provided the means covered by any one of the following claims be employed.

I therefore particularly point out and distinctly claim as my invention—

1. In the art of copper separation, the proc-

- 23
- ess which consists in: first, treating copper-nickel matte to form copper-nickel alloy substantially free from sulfur; then, treating said alloy with chlorin and a solvent for cuprous chlorid, substantially as set forth. 5
2. In the art of copper separation, the process which consists in: subjecting a mass of cupriferous material to chlorin introduced at one point of said mass, and concurrently subjecting said mass to a solvent for cuprous chlorid introduced at another point of said mass, substantially as set forth. 10
3. In the art of copper separation, the process which consists in: treating copper-nickel matte to form copper-nickel alloy substantially free from sulfur; subjecting a mass of said alloy to chlorin introduced at one point of said mass, and concurrently subjecting said mass to a solvent for cuprous chlorid introduced at another point of said mass, substantially as set forth. 15
4. In the art of copper separation, the process which consists in: subjecting a mass of cupriferous material to chlorin introduced therein below the top of said mass, and concurrently subjecting said mass to a solvent for cuprous chlorid introduced therein at a higher level than said chlorin is introduced, substantially as set forth. 20
5. In the art of copper separation, the process which consists in: treating copper-nickel matte to form copper-nickel alloy substantially free from sulfur; subjecting a mass of said alloy to chlorin introduced therein below the top of said mass, and concurrently subjecting said mass to a solvent for cuprous chlorid introduced therein at a higher level than said chlorin is introduced, substantially as set forth. 25
6. In the art of copper separation, the process which consists in: subjecting copper-nickel alloy to chlorin and a solvent for cuprous chlorid, thereby forming a solution of copper chlorid and nickel chlorid; electrolyzing said solution, plating out copper therefrom, and forming a residuary solution of nickel chlorid; electrolyzing said solution of nickel chlorid, plating out nickel therefrom, and separating chlorin therefrom, substantially as set forth. 30
7. In the art of copper separation, the process which consists in: treating copper-nickel matte to form copper-nickel alloy substantially free from sulfur; subjecting said alloy to chlorin and a solvent for cuprous chlorid, thereby forming a solution of copper chlorid and nickel chlorid; electrolyzing said solution, plating out copper therefrom, and forming a residuary solution of nickel chlorid; electrolyzing said solution of nickel chlorid, plating out nickel therefrom, and separating chlorin therefrom, substantially as set forth. 35
8. In the art of copper separation, the process which consists in: electrolyzing a solution of copper chlorid and nickel chlorid, plating out nickel therefrom, and forming a residuary solution of nickel chlorid; electrolyzing said solution of nickel chlorid, plating out nickel therefrom, and separating chlorin therefrom; subjecting cupriferous material to the concurrent action of said chlorin and a solvent for cuprous chlorid, substantially as set forth. 40
9. In the art of copper separation, the process which consists in: electrolyzing a solution of copper chlorid and nickel chlorid, plating out nickel therefrom, and forming a residuary solution of nickel chlorid; electrolyzing said solution of nickel chlorid, plating out nickel therefrom, and separating chlorin therefrom; subjecting copper-nickel matte to form copper-nickel alloy substantially free from sulfur; subjecting said alloy to the concurrent action of said chlorin and a solvent for cuprous chlorid, substantially as set forth. 45
10. In the art of copper separation, the process which consists in: electrolyzing a solution of nickel chlorid, plating out nickel therefrom, and separating chlorin therefrom; subjecting cupriferous material concurrently to said chlorin and a solvent for cuprous chlorid, substantially as set forth. 50
11. In the art of copper separation, the process which consists in: electrolyzing a solution of nickel chlorid, plating out nickel therefrom, and separating chlorin therefrom; treating copper-nickel matte to form copper-nickel alloy substantially free from sulfur; subjecting said alloy concurrently to said chlorin and a solvent for cuprous chlorid, substantially as set forth. 55
12. In the art of copper separation, the process which consists in: electrolyzing a solution of nickel chlorid, plating out nickel therefrom, and separating chlorin therefrom; subjecting copper-nickel alloy concurrently to said chlorin and a solvent for cuprous chlorid; electrolyzing the residuary solution of copper chlorid and nickel chlorid, plating out copper therefrom, and leaving nickel-chlorid solution, substantially as set forth. 60
13. In the art of copper separation, the process which consists in: electrolyzing a solution of nickel chlorid, plating out nickel therefrom, and separating chlorin therefrom; treating copper-nickel matte to form copper-nickel alloy substantially free from sulfur; subjecting said alloy concurrently to said chlorin and a solvent for cuprous chlorid; electrolyzing the residuary solution of copper chlorid and nickel chlorid, plating out copper therefrom, and leaving nickel-chlorid solution, substantially as set forth. 65